

## UNITED STATES PATENT OFFICE.

ALBERT W. MERRICK, OF SCOTIA, NEW YORK, ASSIGNEE TO GENERAL ELECTRIC COMPANY, A CORPORATION OF NEW YORK.

## PROCESS OF MAKING HEAT-RESISTING ALLOYS.

No Drawing.

Application filed April 7, 1922. Serial No. 550,474.

*To all whom it may concern:*

Be it known that I, ALBERT W. MERRICK, a citizen of the United States, residing at Scotia, county of Schenectady, State of New York, have invented certain new and useful Improvements in Processes of Making Heat-Resisting Alloys, of which the following is a specification.

This invention relates to alloys and more particularly to the formation of alloys containing metals such as aluminum which have a lower melting point than that of the metals with which it is alloyed and have a lower specific gravity than such other metals.

The metal aluminum lends valuable properties to other metals, particularly to the ferrous metals. An alloy of aluminum with iron is heat resistant although if the percentage of aluminum is high enough to make the alloy resistant to high temperatures the alloy becomes quite brittle. It has been found, however, that by adding aluminum to a nickel-iron alloy, the alloy becomes tough and strong and at the same time exceedingly heat resistant. Such an alloy containing 10% of aluminum, 30% of nickel, 5% of chromium and 55% of iron, is described and claimed in an application of Gerald R. Brophy, Serial No. 478,422, filed June 17, 1921, assigned to the same assignee as this application. This alloy is practically inoxidizable at high temperatures.

In the formation of such an alloy a very practical difficulty is encountered due to the lower melting point of the aluminum with reference to the nickel and iron and also due to the lower specific gravity. Aluminum melts at about 1160° F., while iron and nickel melt at approximately 3000° F. The specific gravity of aluminum is about 2.6, while iron and nickel have specific gravities of about 8 or 9.

In view of the great difference in the melting points of aluminum on the one hand and nickel or iron on the other, it is impracticable to melt the three metals together in a furnace. The iron and nickel must be melted separately and the aluminum added thereto. Owing, however, to the low specific gravity of the aluminum, it cannot be effectively introduced into the molten nickel iron from the top since it will merely float on the surface. Upon attempting to pour the molten iron and nickel into a ladle containing molten aluminum, a rapid oxida-

tion of the aluminum—so rapid as to constitute an explosion—occurs. Upon investigation and experiment it was found this was due to the presence of the slag on the molten nickel-iron. Upon skimming off the slag, 60 the molten iron was poured into the ladle containing molten aluminum and the metals mixed very quietly and without oxidation of the aluminum. The rapid oxidation when the slag is on the molten nickel-iron is believed to be due to the affinity of the two slags; namely, the slag on the nickel-iron and the slag or dross on the aluminum. Apparently when the slag on the nickel-iron 65 strikes the slag on the aluminum the latter 70 is quickly drawn off into the other slag leaving a clean surface on the aluminum which at the high temperature of the nickel-iron burns with the force of an explosion.

In the practical application of my process 75 instead of skimming off the slag I employ a "bottom pour" ladle for the molten nickel-iron so that only the clean metal comes into contact with the aluminum with the result that with the aid of stirring a uniform alloy 80 results. I am aware that the use of a "bottom pour" ladle to avoid pouring off the slag into a mold is well known and commonly used. So far as I am aware, however, 85 I am the first to recognize the fact that the slag on the metal causes the aluminum to be deprived of its protecting slag, and that by not allowing the two slags to come into contact with each other, a molten metal, 90 such as nickel-iron, can be successfully poured onto a molten metal having a much lower melting point, such as aluminum.

What I claim as new and desire to secure by Letters Patent of the United States, is,— 95

1. The process of preventing oxidation of the metal of lower melting point in the formation of alloys containing metals having widely differing melting points, which consists in melting the metals separately and then pouring the metal of higher melting point onto the other metal under conditions which prevent the slags of the two metals from coming into contact.

2. The process of preventing oxidation of the aluminum in the formation of alloys containing aluminum and a second metal having a higher melting point, which consists in melting the metals separately and then pouring the second metal onto the 105 aluminum under conditions which prevent 110

the slags of the two metals from coming into contact.

3. The process of preventing oxidation of the aluminum in the formation of an alloy of aluminum and iron, which consists in melting the aluminum and iron separately and pouring the iron onto the aluminum under conditions which prevent the slags of the two metals from contact.
- 10 4. The process of preventing oxidation of the aluminum in the formation of an alloy of aluminum and nickel iron, which consists in melting the aluminum and nickel iron separately and then pouring the nickel iron onto the aluminum under conditions which prevent the slags of the two metals from contact.
- 15 5. The process of preventing oxidation of the metal of lower melting point in the formation of alloys containing metals having widely differing melting points which

consists in melting the metals separately, placing them in separate ladles, and then pouring the metal of higher melting point from the bottom of its ladle onto the other metal.

6. The process of preventing oxidation of the aluminum in the formation of an alloy of aluminum and iron which consists in melting the aluminum and iron separately and pouring the iron from the bottom of a ladle onto the aluminum.

7. The process of preventing oxidation of the aluminum in the formation of an alloy of aluminum and nickel iron, which consists in melting the aluminum and nickel iron separately and then pouring the nickel iron from the bottom of a ladle onto the aluminum.

In witness whereof I have hereunto set my hand this 6th day of April, 1922.

ALBERT W. MERRICK.